

Oct. 9, 1928.

1,687,034

M. H. NEWELL

## PROCESS OF PRODUCING A METAL DUST MIXTURE

Filed April 11, 1927



## UNITED STATES PATENT OFFICE.

MINTON H. NEWELL, OF SAN FRANCISCO, CALIFORNIA, ASSIGNEE TO THE ALLOYS COMPANY, OF SAN FRANCISCO, CALIFORNIA, A CORPORATION OF CALIFORNIA.

## PROCESS OF PRODUCING A METAL-DUST MIXTURE.

Application filed April 11, 1927. Serial No. 182,972.

The invention relates to an improvement in processes of producing a metal dust mixture, and more particularly to an improved process of producing a zinc-lead dust.

5 Metal dust has found wide application in the arts. Usually the dust is composed of the single metal. A demand has grown up, however, for a compound metal dust, that is, a dust composed of two or more 10 metals. For example, a dust composed of zinc with a certain proportion of lead has been found a much more active reagent in precipitating precious metals in the cyanide process, than zinc dust alone. To secure 15 the effect of a combined zinc-lead dust, it has heretofore been the practice to add to the cyanide solution of the precious metals the proper quantity of lead in a soluble form, such as acetate, and then add the 20 zinc dust to the solution. It has been found difficult to regulate properly the amount of lead added to the solution in this manner to effect the desired reaction with the zinc, hence there is a demand in the cyanide 25 process industry for a zinc dust containing the proper proportion of lead. Up to the present time, however, no satisfactory process has been devised for producing a zinc-lead mixture of proper proportions, and of 30 the requisite degree of fineness.

One object of the present invention is to provide a process of producing a metal dust mixture in which the ingredients will be properly proportioned and of the requisite 35 fineness of subdivision. A more specific object of the invention is to produce a zinc-lead dust mixture in which the amount of metallic lead will be properly proportioned to the zinc. To these ends, the invention, 40 in one aspect, consists in producing a metal vapor by heating a metal in a retort to the point of vaporization, and introducing into the hot metal vapor a metalliferous oxide of which the metallic element differs from 45 the metal of the vapor and is capable of releasing oxygen by action of the hot vapor. I prefer to use a metalliferous oxide because I have found by previous experiments (see my U. S. Patent 1,456,035, dated May 22, 50 1923) that the introduction of oxygen in controlled amounts into the metal vapor accelerates the condensation of the vapor and promotes the condensing of the vapor in finer particles than can be secured without

introducing oxygen into the vapor. I have 55 now discovered that by introducing into the metal vapor a finely divided metalliferous oxide containing the metal I desire to mix with the metal to be condensed from the vapor, I can secure substantially the required amount of oxygen to cause the vapor to condense in the requisite degree of fineness, and at the same time obtain a finely divided metallic dust from the decomposed oxide. If the oxide does not contain the 60 proper amount of oxygen to cause the vapor to condense in the requisite degree of fineness, I introduce into the mixture a sufficient additional amount of oxygen from external sources, as from a supply of oxygen maintained for this purpose or from the atmosphere. Metal oxides are also desirable 65 because they can be ground very fine and on decomposition yield a much finer metallic dust than can be obtained by grinding the 70 metal itself.

To produce a zinc-lead mixture, the improved process consists in vaporizing the zinc and introducing into the zinc vapor the proper amount of finely divided lead oxide to give the required amount of metallic lead in the zinc-lead dust mixture. The zinc vapor acts on the lead oxide and decomposes it, forming finely divided metallic lead and liberating oxygen which combines with a portion of the zinc vapor to form zinc oxide. The mixture of zinc vapor, metal lead and zinc oxide is then cooled sufficiently rapidly to cause the zinc vapor to condense in fine particles in intimate contact with the finely divided metallic lead. In practicing the process to produce the lead-zinc dust mixture, I heat the zinc in a retort, the mouth of which discharges into a condensing chamber, the walls of which 85 are preferably composed of some substance which rapidly radiates heat, such as iron or steel. The retort is preferably inclined at an angle upwardly so that it will discharge 90 the stream of zinc vapor or fumes upwardly into the condensing chamber. As the stream of zinc vapor enters the condensing chamber, it becomes cooler and a portion of it condenses out into particles of metallic zinc. Into this stream of zinc vapor entering the 95 condensing chamber from the mouth of the retort I introduce a continuous supply of finely divided lead oxide which is decom- 100 105

posed by the vapor. The mixture of vapor, metallic zinc, metallic lead and zinc oxide is preferably circulated within the condensing chamber to accelerate the condensation. This circulating mixture will in practice receive and carry with it some of the finely divided lead oxide which will thereby be acted upon by the hot zinc vapor and decomposed into the metallic lead and oxygen. If the oxygen introduced into the mixture of vapor and metallic oxide particles in this manner is not sufficient to promote the proper degree of fineness of condensation of the zinc vapor, I then add the required amount of oxygen from an external source.

The improved process in its more specific and preferred form for producing a zinc-lead dust mixture, may be practiced in the apparatus shown in the accompanying drawings of which Fig. 1 is a side elevation of the condensing chamber with its accessory apparatus and showing in section the furnace for heating the zinc and the means for feeding the lead oxide, and Fig. 2 is a top plan of the parts shown in Fig. 1.

The apparatus comprises a retort 1 of usual form located within a furnace 2. The retort 1 is inclined at an angle so that its mouth 3 projects through the wall 4 of the furnace 2 and enters the hood 5 which serves as a connection between the furnace 2 and the condensing chamber or condenser 6. A tight joint 7 is established between the hood 5 and the wall 4 of the furnace 2 by luting the joint. As the vapors from the retort 1 enter the condenser 6 they begin to condense and the mixture of vapor and particles of metal zinc are circulated within the condenser by means of the fan 8 located on top of the condenser. The intake 10 of the fan opens into the condenser, and a discharge pipe 9 is directed downwardly within the condenser, terminating above the mouth 3 of the retort 1, so as to direct the mixture of vapors and metal particles into the hot zone of zinc vapor above the mouth of the retort. The fan 8 is driven by the motor 11.

The finely divided lead oxide is introduced into the upper part of the hood 5 through the discharge opening 12 of a hopper 13 provided with the feed mechanism 14 which may be driven from any convenient source. It is preferred to locate the lead oxide feeding devices in the top of the hood 5 so that as the powdered lead oxide falls down into the hood 5 it may disseminate in the mixture of zinc vapor and metallic zinc particles and be drawn by the steam issuing from the mouth of the discharge pipe 9 into the hot zone of zinc vapor near the mouth 3 of retort 1. Thus there is a constant stream of zinc vapor, particles of metallic zinc and particles of lead oxide entering the hot zinc vapor near the mouth of the retort 1, in which zone the lead oxide is decomposed,

forming metallic lead and liberating oxygen which combines with a portion of the zinc vapor to form zinc oxide. As a result of these reactions,—after the apparatus has been put into full operation,—there is maintained within the condenser 6 a circulation of zinc vapor, particles of metallic zinc, particles of metallic lead and particles of zinc oxide, it being understood that the lead oxide will be decomposed when it is brought within the hot zone near the mouth 3 of the retort 1. To prevent ingress of oxygen into the condenser 6 through the hopper 13, a sufficient amount of lead oxide is maintained within the hopper.

If the oxygen liberated from the lead oxide is not sufficient in quantity to effect the requisite degree of oxidation of the zinc, additional oxygen may be drawn into the mixture within the condenser 6 by means of the breather 15 connected with the condenser by the pipe fitting 16. An additional means of introducing oxygen from the air is provided by the valve controlled pipe 17. Access to the interior of the condenser 6 may be had through the plugged opening 18. As zinc condenses in conjunction with the metallic lead and zinc oxide it falls out of the circulating mixture and accumulates in the cone shaped bottom 19 of the condenser, from which it is withdrawn through the discharge door 20.

It will be understood that by regulating the quantity of finely divided lead oxide relatively to the amount of zinc the resultant dust will contain the desired relative quantities of zinc and lead.

Having thus described the invention, what I claim as new is;

1. The process of producing a zinc-lead dust which consists in vaporizing zinc, decomposing lead oxide in the zinc vapor and then cooling the mixture sufficiently rapidly to condense the zinc in a finely divided condition.

2. The process of producing a zinc-lead dust which consists in vaporizing zinc, introducing lead oxide in finely divided condition into the zinc vapor to produce finely divided metallic lead and liberate oxygen to form zinc oxide, and then cooling the mixture sufficiently rapidly to accelerate the formation of finely divided zinc.

3. In the process of producing a zinc-lead dust, including vaporizing zinc, the steps of simultaneously liberating finely divided metallic lead and oxygen in the zinc vapor, and then cooling the mixture sufficiently rapidly to condense the zinc in a finely divided condition.

4. The process of manufacturing zinc-lead dust which consists in vaporizing zinc, conducting the zinc vapor into a condenser, maintaining a circulation within the condenser, and introducing finely divided lead

oxide into the stream of vapor entering the condenser.

5. In the process of manufacturing zinc-lead dust including producing zinc vapor containing particles of metallic zinc in suspension, the steps of introducing finely divided lead oxide into the mixture of vapor and metallic zinc and then introducing the

mixture so formed into a relatively hot, pure zinc vapor.

6. The process of producing zinc-lead dust which consists in mixing finely divided zinc and finely divided lead oxide at a temperature sufficient to decompose the lead oxide and then cooling the mixture.

MINTON H. NEWELL.